



US006136109A

# United States Patent [19]

Miyata et al.

[11] Patent Number: 6,136,109

[45] Date of Patent: Oct. 24, 2000

[54] **METHOD OF MANUFACTURING HIGH CHROMIUM MARTENSITE STEEL PIPE HAVING EXCELLENT PITTING RESISTANCE**

[75] Inventors: **Yukio Miyata; Mitsuo Kimura; Tomoya Koseki; Takaaki Toyooka; Fumio Murase**, all of Aichi, Japan

[73] Assignee: **Kawasaki Steel Corporation**, Japan

[21] Appl. No.: **09/181,829**

[22] Filed: **Oct. 28, 1998**

## Related U.S. Application Data

[62] Division of application No. 08/634,860, Apr. 19, 1996, Pat. No. 5,858,128.

## Foreign Application Priority Data

Apr. 21, 1995 [JP] Japan ..... 7-097063  
Feb. 23, 1996 [JP] Japan ..... 8-036247

[51] Int. Cl. <sup>7</sup> ..... **C21D 9/08**

[52] U.S. Cl. ..... **148/592**; 148/605

[58] Field of Search ..... 148/592, 605,  
148/611

## References Cited

### U.S. PATENT DOCUMENTS

5,049,210 9/1991 Miyasaka et al. ..... 148/592  
5,858,128 1/1999 Miyata et al. ..... 148/325

## FOREIGN PATENT DOCUMENTS

|          |         |       |       |         |
|----------|---------|-------|-------|---------|
| 60-26616 | 2/1985  | Japan | ..... | 148/605 |
| 5-140645 | 6/1993  | Japan | ..... | 148/592 |
| 5-263137 | 10/1993 | Japan | ..... | 148/592 |
| 6-88130  | 3/1994  | Japan | ..... |         |

Primary Examiner—George Wyszomierski  
Attorney, Agent, or Firm—Austin R. Miller

## [57]

## ABSTRACT

A high-Cr martensite steel pipe having excellent pitting resistance and method for manufacturing the same, which involves forming a pipe of steel including C: about 0.03 wt % or less, Si: about 0.5 wt % or less, Mn: about 0.5–3.0 wt %, Cr: about 10.0–14.0 wt %, Ni: about 0.2–2.0 wt %, Cu: about 0.2–1.0 wt % and N: about 0.03 wt % or less with the balance being Fe and incidental impurities, and having a value X shown as defined in the following formula (1) of about 12.2 or more. The pipe is quenched after austenitizing it at a temperature substantially equal to an  $A_{C3}$  point or higher, and the pipe is annealed in a temperature range from about 550° C. or higher to a temperature lower than an  $A_{C1}$  point.

$$\text{value } X = (Cr\%) + 3(Cu\%) - 3(C\%) \quad (1)$$

The high-Cr martensite steel pipe made by this method exhibits excellent pitting resistance and overall surface corrosion resistance even in an environment containing a carbonic acid gas, and further exhibits excellent weldability and toughness in the welding-heat-affected zones.

**12 Claims, No Drawings**

**METHOD OF MANUFACTURING HIGH CHROMIUM MARTENSITE STEEL PIPE HAVING EXCELLENT PITTING RESISTANCE**

This is a division out of our parent application, Ser. No. 08/634,860, filed Apr. 19, 1996, now U.S. Pat. No. 5,858,128, granted Jan. 12, 1999.

**BACKGROUND OF THE INVENTION**

1. Field of the Invention

The present invention relates to a method for manufacturing a martensite stainless steel pipe having excellent corrosion resistance. The invention may be used in manufacturing petroleum and natural gas pipelines.

2. Description of the Related Art

Almost all of the petroleum and natural gas in the world which can be easily extracted has been recovered. Therefore, more and more development is taking place in severe environments, particularly in wells deep underground, frigid locations and offshore sites.

Significant quantities of carbonic acid gas are often contained in petroleum and natural gas recovered from wells located in these severe environments, thereby causing great corrosion of carbon steel or low alloy steels. To cope with this problem, an inhibitor is conventionally added to such steels as a corrosion prevention means.

However, inhibitors not only increase the cost of the steels, they are not effective at high temperatures. Steels which are corrosion resistant without inhibitors, such as martensite stainless steel containing 13% Cr, are now widely used in place of steels containing inhibitors.

API Standards require that a line pipe be composed of 12% Cr martensite stainless steel containing a reduced amount of C. However, this steel is almost never employed as line pipe because preheating and postheating are required for peripheral welding, which tremendously increases costs. Further, toughness in the welded portions is poor. Consequently, two-phase stainless steel having an increased amount of C as well as Ni and Mo is often used as corrosion resistant line pipe because it possesses excellent weldability and corrosion resistance. However, the two-phase stainless steel is expensive and often exceeds the requirements dictated by conditions in some wells.

A method of manufacturing a martensite stainless steel line pipe is disclosed in, for example, Japanese Patent Application Laid-Open No. 4-99128 as a means for overcoming the above problem. Disclosed therein is a method of manufacturing a line pipe of 13% Cr stainless steel which comprises 1.2-4.5% Cu and reduced contents of C and N. After the 13% Cr stainless steel is formed into a pipe, the pipe is cooled at a quenching cooling speed higher than that effected by water. As a result, the stainless steel pipe exhibits excellent corrosion resistance even in a corrosive environment containing a carbonic acid gas, has low hardness in a welding-heat-affected zone and avoids quench cracking. However, this method still fails to produce sufficient toughness in the welding-heat-affected zone (HAZ zone).

An object of the present invention is to provide a method of manufacturing martensite stainless steel pipe having high surface corrosion resistance, high pitting resistance, excellent weld cracking resistance and welded portion toughness.

**SUMMARY OF THE INVENTION**

We have discovered a method for manufacturing high-Cr martensite stainless steel for line pipe having excellent

corrosion resistance and weldability and, in particular, welding-heat-affected zone toughness, all required in a carbonic acid gas environment. The high-Cr martensite stainless steel made by the invention is produced by applying a proper heat treatment to Cr steel in which C and N contents are each reduced to about 0.03 wt % or less, preferably about 0.02 wt % or less, and Cu content is controlled to about 0.2-0.7 wt %.

That is, the present invention provides a method of manufacturing a high-Cr martensite steel pipe which exhibits excellent pitting resistance, comprising the steps of making a steel pipe from a steel comprising C: about 0.03 wt % or less, Si: about 0.5 wt % or less, Mn: about 0.5-3.0 wt %, Cr: about 10.0-14.0 wt %, Ni: about 0.2-2.0 wt %, Cu: about 0.2-0.7 wt % and N: about 0.03 wt % or less, with the balance being Fe and incidental impurities, and having a value X as defined in the following formula of about 12.2 or more:

$$value X = (Cr\%) + 3(Cu\%) - 3(C\%) \quad (1)$$

quenching the pipe after austenitizing it at a temperature substantially equal to the  $A_{c3}$  point or higher, and annealing the pipe in a temperature range from about 550° C. to lower than the  $A_{c1}$  point.

Further, the invention provides a method of manufacturing a high-Cr martensite steel pipe having excellent pitting resistance, wherein after the above-described steel is formed into a steel pipe, the steel pipe is quenched after it is austenitized at a temperature substantially equal to the  $A_{c3}$  point or higher, followed by air cooling the steel pipe.

The present invention further provides a method of manufacturing a high-Cr martensite steel pipe having excellent pitting resistance, wherein after the above-described steel is formed into a steel pipe, the steel pipe is quenched after it is austenitized at a temperature substantially equal to the  $A_{c3}$  point or higher, thereafter the steel pipe is heat treated by maintaining the steel pipe in a temperature range from the  $A_{c1}$  point to the  $A_{c1}$  point+about 50° C. for about 10-60 minutes. The steel pipe is subsequently cooled and annealed at a temperature lower than the  $A_{c1}$  point.

Further, according to the present invention, there is provided a method of making high-Cr martensite steel pipe having excellent pitting resistance, formed from a steel comprising C: about 0.03 wt % or less, Si: about 0.5 wt % or less, Mn: about 0.5-3.5 wt %, Cr: about 10.0-14.0 wt %, Ni: about 0.2-2.0 wt %, Cu: about 0.2-0.7 wt % and N: about 0.03 wt %, with the balance being Fe and incidental impurities, and having a value X as defined in the following formula of about 12.2 or higher:

$$value X = (Cr\%) + 3(Cu\%) - 3(C\%) \quad (1)$$

Further, the invention provides a method of making a high-Cr martensite steel pipe having excellent pitting resistance, made from a steel which, in addition to the above-described components, further comprises at least one element selected from Ti, V, Zr, Nb and Ta in a total amount of about 0.3 wt % or less, and having a value Y as defined in the following formula (2) of about 12.2 or more:

$$value Y = (Cr\%) + 3(Cu\%) - 3(C\%) + (Ti\%) + (V\%) + (Zr\%) + (Nb\%) + (Ta\%) \quad (2)$$

Other embodiments and equivalents of the present invention will become apparent from the following detailed description.

## DETAILED DESCRIPTION OF THE INVENTION

The components and associated content limits of the martensite stainless steel made by the method of the present invention will now be described.

C: about 0.03 wt % or less

C content is preferably reduced as much as possible in order to reduce the hardness of the welding-heat-affected zone, enhance toughness and welding crack resistance, and to increase the corrosion resistance and pitting resistance in a carbonic acid gas environment. C content must be controlled to about 0.03 wt % or less to permit welding of the stainless steel without preheating, and is preferably controlled to about 0.02 wt % or less.

Si: about 0.5 wt % or less

Si is present in the composition of the method as a deoxidizing element. However, since Si promotes the creation of ferrite, excessive amounts of Si increase ferrite content in the steel and deteriorate the toughness of the steel and welded portions thereof. In addition, the presence of ferrite can render seamless steel pipe production difficult. Thus, Si content is controlled to about 0.5 wt % or less and preferably about 0.3 wt % or less.

Mn: about 0.5–3.0 wt %

Mn is required in the method of the invention to promote deoxidation and increase strength. Further, since Mn is an austenite creating element, it acts to suppress the creation of ferrite and improve the toughness of the steel and the welded portions thereof. Mn provides these benefits when at least about 0.5 wt % is present. The benefits provided by Mn do not further accrue when contents exceed about 3.0 wt %, thus Mn content is controlled to about 0.5–3.0 wt % and preferably about 0.8–2.7 wt %.

Cr: about 10–14 wt %

Cr is required in the invention to produce a martensite structure and promote corrosion resistance to carbonic acid gas. About 10 wt % or more Cr must be present to obtain these benefits. On the other hand, if Cr content exceeds about 14 wt %, the creation of ferrite is promoted. Consequently, a large amount of an austenite-promoting element must be added to stably obtain the martensite structure, thereby increasing costs. Thus, Cr content is controlled to about 10–14 wt %.

Ni: about 0.2–2.0 wt %

Ni serves as an austenite-promoting element in the present invention which compensates for the reduction of C and N. Ni also improves the corrosion resistance and toughness of a steel in a carbonic acid gas environment. To realize these benefits, Ni content must be about 0.2 wt % or more. However, if the Ni content exceeds about 2.0 wt %, the  $A_{c1}$  point is lowered such that annealing must be effected for an extended time, thereby inflating production costs. Thus, Ni content is controlled to about 0.2–2.0 wt % and preferably about 0.5–1.7 wt %. Cu: about 0.2–0.7 wt %

Cu compensates for the reduction of C and N by acting as an austenite-promoting element together with Ni and Mn. Cu also improves toughness in the welding-heat-affected zone and promotes corrosion resistance to carbonic acid gas. Cu content must be about 0.2 wt % or more to realize these benefits. However, Cu contents exceeding about 1.0 wt % cause partial precipitation of Cu (i.e., some Cu is not dissolved in solid) and adversely affects the toughness of the steel and the welding-heat-affected zone. Thus, Cu content ranges from about 0.2–0.7 wt %.

N: about 0.03 wt % or less

N content is preferably minimized like that of C to reduce hardness and enhance the toughness of the welding-heat-

affected zone, as well as to promote weld cracking resistance. When N content exceeds about 0.03%, weld cracking occurs and welding-heat-affected zone toughness deteriorates. Therefore, N content is controlled to about 0.03% or less and preferably about 0.02% or less. Total content Ti, V, Zr, Ta: about 0.3% or less

Ti, V, Zr, Ta each have a strong affinity for C and a strong carbide-forming tendency. Cr carbide is replaced with Ti, V, Zr and/or Ta carbide by adding at least one of Ti, V, Zr, Ta. Through these additions, Cr carbide content is reduced, thereby effectively increasing the amount of Cr available to enhance corrosion resistance and pitting resistance of the steel.

Although Ti, V, Zr, Ta improve the toughness of the steel and the welding-heat-affected zone, when their total quantity exceeds about 0.3%, weld cracking sensitivity increases and toughness deteriorates. Thus, the upper total content limit is controlled to about 0.3%.

It is preferable that the Ti content be about 0.01–0.2%, V content be about 0.01–0.1%, Zr content be about 0.01–0.1%, and Ta content be about 0.01–0.1%. When added in composite, their total content is preferably about 0.03–0.2%.

Although the other elements may be incidentally contained in the invention, their content is preferably reduced as much as possible. For example, although the maximum contents of P and S are about 0.03 wt % and about 0.01 wt %, respectively, it is preferable to reduce these amounts as much as possible. A content of O is permitted up to about 0.01 wt %.

value X: about 12.2 or more

$$\text{value } X = (Cr\%) + 3(Cu\%) - 3(C\%) \quad (1)$$

$$\text{value } Y = (Cr\%) + 3(Cu\%) - 3(C\%) + (Ti\%) + (V\%) + (Zr\%) + (Ta\%) \quad (2)$$

The value X is an index for evaluating pitting resistance in an environment containing a carbonic acid gas. We discovered that when the index is about 12.2 or more, no pitting occurs even when a steel is exposed to a 20% NaCl solution in which carbonic acid gas of 3.0 MPa is saturated. Since pitting occurs when the value X is less than about 12.2, the lower limit of the value X is about 12.2. When the value X is too high, martensite structure is difficult to obtain. Therefore, the value X preferably ranges from about 12.2–14.2.

In the method of the invention, stainless steel having the above composition is prepared in a converter or an electric furnace and is solidified by continuous casting or other known casting methods. Molten steel may be refined in a ladle, degassed in vacuum, or subjected to other processings when necessary.

A steel made by the method in accordance with the invention is formed into a pipe through known seamless steel pipe making methods such as the plug mill method, the mandrel mill method or the like, or through known welded steel pipe manufacturing methods like those used in the production of electroseamed steel pipe, UOE steel pipe, and spiral steel pipe, for example. Thereafter, the steel pipe is subjected to a heat treatment(s), wherein the steel pipe is austenitized at a temperature substantially equal to the  $A_{c3}$  point or higher and then quenched.

The austenitization is effected at a temperature substantially equal to the  $A_{c3}$  point or higher to make the steel structure uniform and provide the steel pipe with predetermined characteristics. However, when the austenitization is effected at an excessively high temperature, particles are roughened, toughness deteriorates and energy costs increase. Thus, the temperature for the austenitization is controlled to

substantially the  $A_{c3}$  point or higher, and preferably in the temperature range of the  $A_{c3}$  point to the  $A_{c1}$  point+about 100° C. Importantly, a steel made according to the present invention can possess a single phase martensite structure by being air-cooled after austenitization.

The above heat treatment effected after quenching is important to achieving the advantageous characteristics of the present invention. The following three types of methods (1), (2), (3) can be applied in accordance with the invention.

(1) Annealing effected at about 500° C. or higher to a temperature lower than the  $A_{c1}$  point

Since the steel pipe is made to a uniformly annealed martensite structure by being annealed in a temperature range from about 500° C. to lower than the  $A_{c1}$  point, excellent toughness can be obtained. When the annealing temperature is lower than about 500° C., annealing is insufficiently effected and adequate toughness cannot be obtained.

Importantly, the steel pipe is preferably held for about 10 minutes or longer in the above temperature range during the annealing process, and the steel pipe may be air-cooled after it is annealed in accordance with the invention.

(2) Heat treatment effected in a temperature range from the  $A_{c1}$  point to the  $A_{c1}$  point+about 50° C. (heat treatment in a two-phase region)

A steel made pipe in accordance with the invention is made to a fine two-phase structure composed of martensite and austenite by being subjected to a heat treatment at the  $A_{c1}$  point or higher and made to a fine martensite structure by being cooled thereafter. Although fresh martensite which is not annealed is mixed in the structure, the fine structure increases toughness. However, when a steel pipe is subjected to a heat treatment at a temperature exceeding the  $A_{c1}$  point+about 50° C., particles are roughened and toughness deteriorates.

The steel pipe is preferably held between about ten minutes to 60 minutes in this temperature range, and thereafter may be air-cooled.

(3) Heat treatment effected in a temperature range from the  $A_{c1}$  point to the  $A_{c1}$  point+about 50° C., and annealing effected thereafter at a temperature substantially equal to the  $A_{c1}$  point or lower

When steel having a structure resulting from heat treatment in accordance with the above item (2) is thereafter annealed, a fine annealed martensite structure can be obtained. Thus a steel pipe having higher toughness results.

The holding time in the respective temperature ranges in the item (3) is the same as those described for the above items (1) and (2), and the steel pipe may be air-cooled after it is held for the periods described above.

Which heat treatment(s) are used may be determined by considering the characteristics required and the manufacturing costs.

The invention will now be described through illustrative examples. The examples are not intended to limit the scope of the appended claims.

#### EXAMPLE 1

5 Steels having compositions as shown in Table 1 were prepared and formed into seamless steel pipes each having a wall thickness of 0.5" (12.7 mm). Subsequently, the steel pipes were subjected to a heat treatment at temperatures also shown in Tables 1-(1) (Examples of the Invention) and 1-(2) (Comparative Examples). Q in Table 1 represents quenching temperatures for austenitization,  $T_d$  represents two-phase region heat treatment temperatures and T represents annealing temperatures equal to or lower than the  $A_{c1}$  point. The holding time for these heat treatments was thirty minutes, and cooling was effected by air in all cases. Joints were formed through peripheral welding utilizing a TIG welding method (neither preheating nor post-heat was effected).

10 Test pieces were collected from the thusly obtained welded joints and a Charpy test was performed on the welding-heat-affected zones of the test pieces. The welded portions of the test pieces were exposed to carbonic acid gas to evaluate corrosion resistance.

15 The Charpy test involved collecting full-size test pieces from the heat-affected zones of the test pieces and measuring absorbed energies at 0° C. The corrosion test involved

20 preparing test pieces of 3.0 mm×25 mm×50 mm to include welded and non-welded portions, dipping the test pieces into a 20% NaCl solution in which a carbonic acid gas of 3.0 MPa was saturated, and holding the test pieces in that corrosive environment for seven days at 80° C. using an autoclave. The corrosion rates of 0.1 mm/year or less of 25 mother material, including welded portions, immersed in a corrosion test liquid of 20% NaCl solution in which a carbonic gas of 3.0 MPa was saturated at 80° C. were evaluated by comparing their measured weights before and 30 after the test, and converting the differences into projected thickness reductions over one year. The results of the test are 35 shown in Tables 1-(1) and 1-(2).

40 As seen in Table 1-(1) the steel pipes made in accordance with the method of the present invention have absorbed energy for heat-affected welding portion of  $\sqrt{E_o} \leq 170$  J at 0° C. The examples of the invention exhibit excellent toughness. In addition, the corrosion rates are 0.1 mm/y or slower in the examples of the invention, which is well within tolerances expected of a corrosion resistant material in practical use. Moreover, no selective corrosion affected the 45 welded portions, and the steel pipes in accordance with the invention demonstrated excellent corrosion resistance to the carbonic acid gas. Since neither preheating nor postheating was necessary to perform the welding, it is apparent that the steel pipes in accordance with the invention also have excellent weldability.

50 Test results for the Comparative Examples were inferior to those of Examples of the Invention, as seen in Table 1-(2).

TABLE 1-(1)

| Examples of the Invention |                             |      |      |      |      |      |       |                             |                             |                    |     |       |      |                    |
|---------------------------|-----------------------------|------|------|------|------|------|-------|-----------------------------|-----------------------------|--------------------|-----|-------|------|--------------------|
| No.                       | Chemical Composition (wt %) |      |      |      |      |      |       | $A_{c1}$<br>Point<br>(° C.) | $A_{c3}$<br>Point<br>(° C.) | Heat Treatment     |     |       | (*1) | (*2)<br>(mm/<br>y) |
|                           | C                           | Si   | Mn   | Cr   | Ni   | Cu   | N     |                             |                             | Temperature (° C.) | Q   | $T_d$ | T    |                    |
| 1                         | 0.010                       | 0.21 | 1.49 | 12.1 | 0.25 | 0.25 | 0.009 | 750                         | 860                         | 1000               | —   | 700   | 180  | 0.072              |
| 2                         | 0.025                       | 0.20 | 1.52 | 12.0 | 0.25 | 0.24 | 0.011 | 730                         | 840                         | 1000               | —   | 700   | 170  | 0.084              |
| 3                         | 0.011                       | 0.20 | 1.51 | 11.9 | 1.02 | 0.24 | 0.011 | 700                         | 810                         | 950                | —   | 650   | 220  | 0.054              |
| 4                         | 0.012                       | 0.19 | 1.48 | 12.0 | 0.24 | 0.51 | 0.012 | 740                         | 850                         | 1000               | —   | 700   | 195  | 0.082              |
| 5                         | 0.011                       | 0.18 | 1.47 | 11.9 | 1.03 | 0.49 | 0.011 | 700                         | 810                         | 950                | —   | 650   | 202  | 0.056              |
| 6                         | 0.011                       | 0.18 | 1.47 | 11.9 | 1.03 | 0.49 | 0.011 | 700                         | 810                         | 950                | 715 | —     | 221  | 0.061              |

TABLE 1-(1)-continued

| No. | Chemical Composition (wt %) |      |      |      |      |      |       | $A_{c1}$<br>Point | $A_{c3}$<br>Point | Heat Treatment     |     |       | (*1) | (*2)<br>(mm/ |
|-----|-----------------------------|------|------|------|------|------|-------|-------------------|-------------------|--------------------|-----|-------|------|--------------|
|     | C                           | Si   | Mn   | Cr   | Ni   | Cu   | N     |                   |                   | Temperature (° C.) | Q   | $T_d$ | T    |              |
| 7   | 0.011                       | 0.18 | 1.47 | 11.9 | 1.03 | 0.49 | 0.011 | 700               | 810               | 950                | 715 | 650   | 254  | 0.055        |
| 8   | 0.012                       | 0.21 | 1.51 | 11.1 | 0.25 | 0.26 | 0.010 | 750               | 840               | 950                | —   | 700   | 195  | 0.092        |
| 9   | 0.010                       | 0.18 | 1.49 | 10.9 | 0.49 | 0.51 | 0.009 | 740               | 820               | 950                | —   | 700   | 213  | 0.089        |
| 10  | 0.010                       | 0.03 | 1.81 | 12.1 | 0.23 | 0.26 | 0.011 | 740               | 850               | 1000               | —   | 700   | 230  | 0.074        |
| 11  | 0.023                       | 0.21 | 1.49 | 12.9 | 1.50 | 0.50 | 0.009 | 680               | 800               | 1000               | —   | 650   | 180  | 0.045        |

(\*1) Energy absorbed by welding-heat-affected Zone

(\*2) Corrosion rate

TABLE 1-(2)

| No. | Chemical Composition (wt %) |      |      |      |      |      |       | $A_{c1}$<br>Point | $A_{c3}$<br>Point | Heat Treatment     |     |       | (*1) | (*2)<br>(mm/     |
|-----|-----------------------------|------|------|------|------|------|-------|-------------------|-------------------|--------------------|-----|-------|------|------------------|
|     | C                           | Si   | Mn   | Cr   | Ni   | Cu   | N     |                   |                   | Temperature (° C.) | Q   | $T_d$ | T    | $\sqrt{E_o}$ (J) |
| 12  | 0.036                       | 0.20 | 1.52 | 12.0 | 0.29 | 0.28 | 0.010 | 730               | 840               | 1000               | —   | 700   | 125  | 0.084            |
| 13  | 0.021                       | 0.20 | 1.52 | 12.0 | —    | 0.21 | 0.010 | 780               | 920               | 1000               | —   | 700   | 132  | 0.084            |
| 14  | 0.230                       | 0.20 | 1.49 | 11.9 | 0.31 | —    | 0.013 | 730               | 840               | 1000               | —   | 700   | 135  | 0.084            |
| 15  | 0.010                       | 0.19 | 1.49 | 8.9  | 0.21 | 0.23 | 0.015 | 740               | 850               | 950                | —   | 700   | 203  | 0.541            |
| 16  | 0.010                       | 0.21 | 1.48 | 14.8 | 1.52 | 0.20 | 0.012 | 780               | 890               | 1000               | —   | 700   | 85   | 0.041            |
| 17  | 0.010                       | 0.71 | 1.51 | 12.1 | 0.23 | 0.31 | 0.009 | 720               | 830               | 1000               | —   | 700   | 92   | 0.070            |
| 18  | 0.012                       | 0.21 | 0.31 | 12.1 | 0.25 | 0.30 | 0.010 | 800               | 900               | 1000               | —   | 600   | 86   | 0.068            |
| 19  | 0.010                       | 0.22 | 1.50 | 12.5 | 0.21 | 1.50 | 0.011 | 730               | 820               | 1000               | —   | 700   | 97   | 0.075            |
| 20  | 0.010                       | 0.19 | 1.49 | 12.5 | 0.23 | 0.32 | 0.035 | 730               | 840               | 1000               | —   | 700   | 112  | 0.079            |
| 21  | 0.011                       | 0.18 | 1.47 | 11.9 | 1.03 | 0.49 | 0.011 | 700               | 810               | 950                | 760 | —     | 56   | 0.069            |
| 22  | 0.011                       | 0.18 | 1.47 | 11.9 | 1.05 | 0.49 | 0.011 | 700               | 810               | 950                | 760 | 650   | 98   | 0.064            |

(\*1) Energy absorbed by welding-heat-affected Zone

(\*2) Corrosion rate

\*\* Underlines indicate values outside of the range of the invention.

## EXAMPLE 2

Steels having compositions as shown in Tables 2-(1) (Examples of the Invention) and 2-(2) (Comparative Examples) were prepared and formed into slabs by continuous casting, and then hot rolled to form steel sheets 15 mm thick. Thereafter, the steel sheets were heated at 900° C. and quenched by air-cooling, followed by annealing at 680° C. (which was lower than the  $A_{c3}$  point).

After the sheets were welded together, an oblique Y-shaped weld cracking test in accordance with JIS Z3158 was performed on these steel sheets at a preheating temperature of 30° C. to evaluate the resistance to weld cracking. Steel sheets which exhibited weld cracking are marked with an "X" and those which exhibited no weld cracking are marked with "O" in Tables 3-(1) (Examples of the Invention) and 3-(2) (Comparative Examples). The welded joints were formed between the steel sheets through TIG welding (neither preheating nor postheating was effected). No cross-sectional cracking was observed.

A Charpy impact test was performed on the welding-heat-affected zones of the joints. A heat input of 15 kJ/cm was used, and the test pieces were collected from the heat-affected zones in accordance with JIS 4 (notch position: 1 mm apart from a bonded portion), and absorbed energies were measured at 0° C.

Further, all of the steel sheets were exposed to carbonic acid gas to evaluate pitting resistance and surface corrosion

resistance. The test was performed by preparing steel test pieces of 3.0 mm×25 mm×50 mm, dipping the pieces into an autoclave containing a 20% NaCl solution in which a carbonic acid gas of 3.0 MPa was saturated, and holding the test pieces therein at 80° C. for seven days.

Pitting resistance was evaluated by washing the exposed test pieces with water and then drying, followed by observation with the naked eye to determine whether pits were formed on the surfaces. Test pieces exhibiting one or more pits were marked with an "x" while those with no pits were marked with an "o" in Tables 3-(1) and 3-(2).

Surface corrosion resistance was evaluated after washing the test pieces with water followed by drying. Subsequently, the weights of the test pieces were measured and compared with their original weights. The rate at which the weights were reduced were converted into thickness reductions projected over a one year period, and the results of these tests are shown in Tables 3-(1) and 3-(2).

As seen in Table 3-(1), weld cracking was not observed in the Examples of the present invention even at the preheating temperature of 30° C., thus confirming the excellent weld cracking resistance of the invention. Further, since the Examples of the Invention had energies of 180 J or more absorbed by the HAZ zones at 0° C., excellent toughness in the welding-heat-affected zones was demonstrated. Further, the Examples of the Invention experienced no pitting and a corrosion speed of 0.1 mm/year or slower, which reveals the

excellent pitting resistance and overall surface corrosion resistance of the invention.

The Comparative Examples were not in accordance with the present invention and exhibited characteristics inferior to

those Examples produced in accordance with the present invention. Specifically, the Comparative Examples exhibited weld cracking, low toughness in HAZ zones, pitting and the like as shown in Table 3-(2).

TABLE 2-(1)

| No. | C     | Si   | Mn   | Cr   | Ni   | Cu   | N     | total from Ti to Ta         |       |       |       |       |       | Value x |       |
|-----|-------|------|------|------|------|------|-------|-----------------------------|-------|-------|-------|-------|-------|---------|-------|
|     |       |      |      |      |      |      |       | Examples of the Invention   |       |       |       |       |       |         |       |
|     |       |      |      |      |      |      |       | Chemical Composition (wt %) |       |       |       |       |       |         |       |
| No. | C     | Si   | Mn   | Cr   | Ni   | Cu   | N     | Ti                          | V     | Zr    | Nb    | Ta    | total | Value x |       |
| 1   | 0.011 | 0.20 | 1.51 | 12.0 | 1.03 | 0.51 | 0.010 |                             |       |       |       |       | —     | 13.50   |       |
| 2   | 0.010 | 0.19 | 1.49 | 11.0 | 0.80 | 0.51 | 0.009 | 0.020                       | 0.059 |       |       |       | —     | 12.50   |       |
| 3   | 0.010 | 0.21 | 1.49 | 12.1 | 1.02 | 0.49 | 0.009 | 0.020                       | 0.059 |       |       |       | 0.079 | 13.62   |       |
| 4   | 0.018 | 0.20 | 1.49 | 12.0 | 0.81 | 0.51 | 0.011 |                             | 0.042 |       |       |       | 0.042 | 13.52   |       |
| 5   | 0.011 | 0.19 | 1.53 | 11.9 | 0.82 | 0.50 | 0.025 | 0.030                       |       |       | 0.050 |       | 0.080 | 13.45   |       |
| 6   | 0.010 | 0.18 | 1.50 | 10.9 | 0.79 | 0.49 | 0.012 |                             | 0.071 | 0.020 |       |       | 0.091 | 12.43   |       |
| 7   | 0.011 | 0.20 | 1.49 | 12.9 | 0.50 | 0.28 | 0.011 | 0.050                       | 0.045 |       |       |       | 0.095 | 13.80   |       |
| 8   | 0.009 | 0.18 | 1.52 | 11.2 | 0.27 | 0.49 | 0.012 | 0.030                       | 0.049 |       |       |       | 0.030 | 0.109   | 12.75 |
| 9   | 0.018 | 0.21 | 1.52 | 11.0 | 0.80 | 0.40 | 0.011 |                             | 0.051 |       | 0.040 |       | 0.091 | 12.24   |       |
| 10  | 0.010 | 0.19 | 1.47 | 11.9 | 0.98 | 0.25 | 0.011 | 0.020                       | 0.051 |       |       |       | 0.071 | 12.69   |       |
| 11  | 0.011 | 0.21 | 1.52 | 11.8 | 0.80 | 0.39 | 0.012 | 0.105                       | 0.042 |       |       |       | 0.147 | 13.08   |       |
| 12  | 0.013 | 0.19 | 1.47 | 12.1 | 0.85 | 0.52 | 0.011 |                             | 0.045 |       | 0.015 | 0.043 | 0.103 | 13.72   |       |
| 13  | 0.012 | 0.18 | 1.51 | 11.8 | 0.79 | 0.55 | 0.015 | 0.021                       | 0.035 | 0.035 | 0.020 |       | 0.111 | 13.53   |       |

TABLE 2-(2)

| No. | C     | Si   | Mn   | Cr   | Ni   | Cu   | N     | total from Ti to Ta         |       |    |       |    |       | Value x |  |
|-----|-------|------|------|------|------|------|-------|-----------------------------|-------|----|-------|----|-------|---------|--|
|     |       |      |      |      |      |      |       | Examples of the Invention   |       |    |       |    |       |         |  |
|     |       |      |      |      |      |      |       | Chemical Composition (wt %) |       |    |       |    |       |         |  |
| No. | C     | Si   | Mn   | Cr   | Ni   | Cu   | N     | Ti                          | V     | Zr | Nb    | Ta | total | Value x |  |
| 14  | 0.025 | 0.21 | 1.49 | 11.8 | 0.99 | 0.58 | 0.016 | 0.015                       | 0.042 |    |       |    | 0.057 | 13.52   |  |
| 15  | 0.012 | 0.19 | 1.51 | 11.9 | 0.98 | 0.49 | 0.038 |                             | 0.049 |    |       |    | 0.049 | 13.38   |  |
| 16  | 0.011 | 0.20 | 1.52 | 9.2  | 1.20 | 0.63 | 0.012 |                             | 0.054 |    |       |    | 0.054 | 11.11   |  |
| 17  | 0.012 | 0.19 | 1.50 | 14.1 | 0.75 | 0.45 | 0.011 | 0.015                       | 0.045 |    | 0.025 |    | 0.085 | 15.50   |  |
| 18  | 0.011 | 0.22 | 1.48 | 12.1 | 0.01 | 0.54 | 0.013 | 0.021                       | 0.035 |    |       |    | 0.056 | 13.74   |  |
| 19  | 0.012 | 0.19 | 1.51 | 11.9 | 1.01 | 1.52 | 0.011 | 0.015                       | 0.045 |    |       |    | 0.060 | 16.48   |  |
| 20  | 0.010 | 0.22 | 1.49 | 12.1 | 1.02 | 0.46 | 0.013 | 0.172                       | 0.088 |    | 0.085 |    | 0.345 | 13.80   |  |
| 21  | 0.015 | 0.23 | 1.49 | 11.7 | 1.10 | 0.11 | 0.011 | 0.015                       | 0.068 |    |       |    | 0.083 | 12.07   |  |
| 22  | 0.019 | 0.19 | 1.50 | 11.1 | 0.89 | 0.30 | 0.012 | 0.023                       | 0.051 |    |       |    | 0.074 | 12.02   |  |

TABLE 3-(1)

| No. | Characteristics of mother material |          |                  |       |          |          | Welding | $\sqrt{E_o}$ of welding-heat-affected zone (J) | Corrosion speed |  |       |  |  |
|-----|------------------------------------|----------|------------------|-------|----------|----------|---------|------------------------------------------------|-----------------|--|-------|--|--|
|     | YS (MPa)                           | TS (MPa) | $\sqrt{E_o}$ (J) | crack | Pitting  |          |         |                                                | (mm/Y)          |  |       |  |  |
|     |                                    |          |                  |       | zone (J) | zone (J) |         |                                                |                 |  |       |  |  |
| No. | YS (MPa)                           | TS (MPa) | $\sqrt{E_o}$ (J) | crack | zone (J) | zone (J) |         |                                                |                 |  |       |  |  |
| 1   | 605                                | 710      | 265              | ○     | 220      | ○        |         |                                                |                 |  | 0.069 |  |  |
| 2   | 593                                | 705      | 272              | ○     | 231      | ○        |         |                                                |                 |  | 0.084 |  |  |
| 3   | 620                                | 732      | 255              | ○     | 205      | ○        |         |                                                |                 |  | 0.072 |  |  |
| 4   | 595                                | 700      | 265              | ○     | 185      | ○        |         |                                                |                 |  | 0.085 |  |  |
| 5   | 600                                | 715      | 252              | ○     | 195      | ○        |         |                                                |                 |  | 0.078 |  |  |
| 6   | 625                                | 730      | 283              | ○     | 214      | ○        |         |                                                |                 |  | 0.085 |  |  |
| 7   | 615                                | 720      | 272              | ○     | 188      | ○        |         |                                                |                 |  | 0.051 |  |  |
| 8   | 580                                | 703      | 293              | ○     | 203      | ○        |         |                                                |                 |  | 0.089 |  |  |
| 9   | 575                                | 695      | 275              | ○     | 196      | ○        |         |                                                |                 |  | 0.088 |  |  |
| 10  | 593                                | 703      | 269              | ○     | 230      | ○        |         |                                                |                 |  | 0.069 |  |  |
| 11  | 607                                | 723      | 273              | ○     | 193      | ○        |         |                                                |                 |  | 0.078 |  |  |
| 12  | 587                                | 693      | 292              | ○     | 223      | ○        |         |                                                |                 |  | 0.073 |  |  |
| 13  | 593                                | 704      | 280              | ○     | 215      | ○        |         |                                                |                 |  | 0.080 |  |  |

TABLE 3-(2)

| Example of the invention |                                    |          |         |                                                |                 |         |
|--------------------------|------------------------------------|----------|---------|------------------------------------------------|-----------------|---------|
| No.                      | Characteristics of mother material |          | Welding | $\sqrt{E_o}$ of welding heat-affected zone (J) | Corrosion speed |         |
|                          | YS (MPa)                           | TS (MPa) |         |                                                | crack           | Pitting |
| 14                       | 609                                | 725      | 240     | x                                              | 168             | o       |
| 15                       | 582                                | 695      | 200     | x                                              | 112             | o       |
| 16                       | 596                                | 721      | 263     | o                                              | 209             | x       |
| 17                       | 573                                | 699      | 252     | o                                              | 178             | o       |
| 18                       | 595                                | 715      | 205     | o                                              | 131             | o       |
| 19                       | 602                                | 715      | 180     | o                                              | 95              | o       |
| 20                       | 589                                | 702      | 156     | x                                              | 85              | o       |
| 21                       | 601                                | 721      | 273     | o                                              | 211             | x       |
| 22                       | 590                                | 717      | 207     | o                                              | 93              | x       |
|                          |                                    |          |         |                                                |                 | 0.201   |

## EXAMPLE 3

Molten steels having compositions as shown in Table 4 were prepared in a converter and formed into steel pipe materials by continuous casting. The steel pipe materials were formed into 273 mm<sup>2</sup> steel pipes by plug mill rolling. Thereafter, the steel pipes were heated to 900° C. and quenched with water, then heated to 680° C. (which was lower than the  $A_{c1}$  point) and held at that temperature, followed by air-cooling.

Test pieces collected from the steel pipes were subjected to testing to determine their mechanical characteristics and

gas can be provided at a low cost, by which the present invention will greatly contribute to the growth of industries.

Although this invention has been described with reference to specific elements and method steps, equivalent elements and method steps may be substituted, the sequence of the steps may be varied, and certain elements and method steps may be used independently of others. Further, various other elements and control steps may be included, all without departing from the spirit and scope of the invention defined in the appended claims.

TABLE 4

| Chemical Composition (wt %) |       |      |                                                |      |      |         |                          |                     |       |    |    |       |
|-----------------------------|-------|------|------------------------------------------------|------|------|---------|--------------------------|---------------------|-------|----|----|-------|
| No.                         | C     | Si   | Mn                                             | Cr   | Ni   | Cu      | N                        | Total from Ti to Ta |       |    |    |       |
|                             |       |      |                                                |      |      |         |                          | Ti                  | V     | Zr | Nb | Ta    |
| A                           | 0.010 | 0.21 | 1.51                                           | 10.9 | 0.81 | 0.49    | 0.009                    | —                   | —     | —  | —  | —     |
| B                           | 0.011 | 0.20 | 1.52                                           | 11.1 | 1.51 | 0.51    | 0.011                    | 0.035               | 0.031 | —  | —  | 0.066 |
| Mother Material YS          |       |      |                                                |      |      |         |                          | Corrosion speed     |       |    |    |       |
| No.                         | MPa   |      | $\sqrt{E_o}$ of welding-heat-affected zone (J) |      |      | Pitting | Reference                |                     |       |    |    |       |
| A                           | 589   |      | 210                                            |      |      | o       | Example of the invention |                     |       |    |    |       |
| B                           | 605   |      | 223                                            |      |      | o       | Example of the invention |                     |       |    |    |       |

45

corrosion resistance. The corrosion resistance was tested under the same conditions as those of Example 2.

Steel pipe joints were made by the TIG welding (voltage: 16 V, current: 180 A, welding speed: 6.0 cm/min.), and the Charpy test was performed on the HAZ zones (1 mm away from bonded portions).

The results of the tests are shown in Table 4. Since the steel pipes of Example 4 exhibit excellent pitting resistance, overall surface corrosion resistance and toughness in the welding-heat-affected zones, they have characteristics well-adapted for service in pipelines.

As described above, the present invention provides a high-Cr martensite steel pipe which exhibits excellent pitting resistance and overall surface corrosion resistance in an environment containing a carbonic acid gas and, in addition, exhibits excellent weldability and toughness in the welding-heat-affected zones. Consequently, according to the present invention, line pipes for transporting petroleum and natural

What is claimed is:

1. A method of manufacturing a high-Cr martensite steel pipe having excellent pitting resistance and overall corrosion resistance, comprising:

50 forming a pipe from a steel material comprising C: about 0.03 wt % or less, Si: about 0.5 wt % or less, Mn: about 0.5–3.0 wt %, Cr: about 10.0–14.0 wt %, Ni: about 0.2–2.0 wt %, Cu: about 0.2–0.7 wt %, N: about 0.03 wt % or less and the balance being Fe and incidental impurities, wherein a value X defined by the following formula (1):

$$value X = (Cr\%) + 3(Cu\%) - 3(C\%) \quad (1)$$

is about 12.2–14.2;

60 austenitizing said pipe at a temperature substantially equal to the  $A_{C3}$  point or higher; quenching said pipe after austenitizing; and annealing said pipe in a temperature range from about 550° C. to a temperature that is lower than the  $A_{C1}$  point of the steel.

65 2. A method of manufacturing a high-Cr martensite steel pipe according to claim 1, wherein said steel further com-

## 13

prises at least one element selected from the group consisting of Ti, V, Zr, Nb and Ta in a total quantity of about 0.3 wt % or less, and wherein the value Y is defined by the following formula (2):

$$\text{value } Y = (Cr\%) + 3(Cu\%) - 3(C\%) + (Ti\%) + (V\%) + (Zr\%) + (Nb\%) + (Ta\%) \quad (2)$$

is about 12.2 or more.

3. A method of manufacturing a high-Cr martensite steel pipe according to claim 1, wherein said forming of said pipe comprises a method of manufacturing a seamless steel pipe or a welded pipe.

4. A method of manufacturing a high-Cr martensite steel pipe according to claim 2, wherein said forming of said pipe comprises a method of manufacturing a seamless steel pipe or a welded pipe.

5. A method of manufacturing a high-Cr martensite steel pipe having excellent pitting resistance and overall corrosion resistance, comprising:

forming a pipe from a steel comprising C: about 0.03 wt % or less, Si: about 0.5 wt % or less, Mn: about 0.5–3.0 wt %, Cr: about 10.0–14.0 wt %, Ni: about 0.2–2.0 wt %, Cu: about 0.2–0.7 wt %, N: about 0.03 wt % or less and the balance being Fe and incidental impurities, wherein a value X defined by the following formula (1):

$$\text{value } X = (Cr\%) + 3(Cu\%) - 3(C\%) \quad (1)$$

is about 12.2–14.2;

austenitizing said pipe at a temperature substantially equal to an  $A_{C3}$  point or higher;

quenching said pipe after austenitizing; and

heat treating said pipe by maintaining said pipe in a temperature range from the  $A_{C1}$  point to said  $A_{C1}$  point plus about 50° C. for about 10–60 minutes; and

cooling said pipe with air.

6. A method of manufacturing a high-Cr martensite steel pipe according to claim 5, wherein said steel further comprises at least one element selected from the group consisting of Ti, V, Zr, Nb and Ta in a total quantity of about 0.3 wt % or less, and wherein said value Y is defined by the following formula (2):

$$\text{value } Y = (Cr\%) + 3(Cu\%) - 3(C\%) + (Ti\%) + (V\%) + (Zr\%) + (Nb\%) + (Ta\%) \quad (2)$$

7. A method of manufacturing a high-Cr martensite steel pipe according to claim 5, wherein said forming of said pipe

## 14

comprises a method of manufacturing a seamless steel pipe or a welded pipe.

8. A method of manufacturing a high-Cr martensite steel pipe according to claim 6, wherein said forming of said pipe comprises a method of manufacturing a seamless steel pipe or a welded pipe.

9. A method of manufacturing a high-Cr martensite steel pipe having excellent pitting resistance and overall corrosion resistance, comprising:

10. forming a pipe from a steel comprising C: about 0.03 wt % or less, Si: about 0.5 wt % or less, Mn: about 0.5–3.0 wt %, Cr: about 10.0–14.0 wt %, Ni: about 0.2–2.0 wt %, Cu: about 0.2–0.7 wt %, N: about 0.03 wt % or less and the balance being Fe and incidental impurities, wherein a value X defined by the following formula (1):

$$\text{value } X = (Cr\%) + 3(Cu\%) - 3(C\%) \quad (1)$$

is about 12.2–14.2;

austenitizing said pipe at a temperature substantially equal to the  $A_{C3}$  point or higher;

quenching said pipe after austenitizing; and

heat treating said pipe by maintaining said pipe in a temperature range from the  $A_{C1}$  point to said  $A_{C1}$  point plus about 50° C. for about 10–60 minutes;

cooling said pipe with air; and

annealing said pipe at a temperature lower than said  $A_{C1}$  point.

10. A method of manufacturing a high-Cr martensite steel pipe according to claim 9, wherein said steel further comprises at least one element selected from the group consisting of Ti, V, Zr, Nb and Ta in a total quantity of about 0.3 wt % or less, and wherein the value Y is defined by the following formula (2):

$$\text{value } Y = (Cr\%) + 3(Cu\%) - 3(C\%) + (Ti\%) + (V\%) + (Zr\%) + (Nb\%) + (Ta\%) \quad (2)$$

11. A method of manufacturing a high-Cr martensite steel pipe according to claim 9, wherein said forming of said pipe comprises a method of manufacturing a seamless steel pipe or a welded pipe.

12. A method of manufacturing a high-Cr martensite steel pipe according to claim 10, wherein said forming of said pipe comprises a method of manufacturing a seamless steel pipe or a welded pipe.

\* \* \* \* \*